# EUROPEAN PATENT SPECIFICATION

(11) **EP 3 395 997 B1**
(45) Date of publication and mention of the grant of the patent: **02.09.2020**
(21) Application number: 16879212.5
(22) Date of filing: 02.12.2016
(51) Int. Cl.: C22C 38/58, C22C 38/50, C22C 38/48, C22C 38/06, C22C 38/02, C22C 38/00, C22C 38/42, C22C 38/44, C22C 38/46, C21D 8/02, C22C 38/04, C22C 38/54

(54) **LOW-YIELD-RATIO TYPE HIGH-STRENGTH STEEL, AND MANUFACTURING METHOD THEREFOR**
HOCHFESTER STAHL MIT NIEDRIGEM STRECKGRENZENVERHÄLTNIS UND HERSTELLUNGSVERFAHREN DAFÜR
ACIER À HAUTE RÉSISTANCE DE TYPE À FAIBLE RAPPORT D'ÉLASTICITÉ ET SON PROCÉDÉ DE FABRICATION

(30) Priority: 24.12.2015 KR 20150186522
(43) Date of publication of application: 31.10.2018
(73) Proprietor: POSCO, Pohang-si, Gyeongsangbuk-do 37859 (KR)
(72) Inventor: YU, Seng-Ho, Pohang-si, Gyeongsangbuk-do 37877 (KR); JUNG, Mun-Young, Seoul 06194 (KR)
(74) Representative: Potter Clarkson
(86) International application number: PCT/KR2016/014135
(87) International publication number: WO 2017/111345

(56) References cited:
- EP-A1- 2 700 728
- WO-A1-2008/054166
- WO-A1-2014/171062
- JP-A- H0 551 694
- JP-A- S5 597 425
- JP-B1- 5 679 091
- KR-A- 20090 052 950
- KR-A- 20090 052 950
- KR-A- 20140 118 316
- KR-A- 20150 002 958
- KR-A- 20150 002 958
- KR-A- 20150 074 968
- KR-A- 20150 074 968

## Description

### [Technical Field]

The present invention relates to low-yield-ratio type, high-strength steel and a manufacturing method therefor, and more particularly, to low-yield-ratio type, high-strength steel that is appropriate for use as steel for construction due to a low yield ratio and high tensile strength, and a manufacturing method therefor.

### [Background Art]

Recently, according to the trend for extremely tall and long span structures, such as domestic and foreign buildings and bridges, there has been a need to develop extra thick high strength steel. When high strength steel is used, the structures of buildings and bridges are rationalized and lightened due to high allowable stress of the high strength steel and, thus, economical construction is possible and a plate thickness is reduced, thereby allowing machining such as cutting or perforation and welding operations to be easily performed.

When the strength of steel is increased, a yield ratio (yield strength/tensile strength) that is a ratio of tensile strength to yield strength is frequently increased. In this regard, when a yield ratio is increased, a stress difference up to a point in time at which deconstruction occurs from a point in time (yield point) at which plastic deformation occurs is not high and, thus, buildings have a low construction margin for preventing buildings from disintegrating through absorbing energy via deformation and, accordingly, when a large external force, such as that of an earthquake is applied, there is a problem in that it is difficult to ensure safety. Accordingly, steel for construction needs to satisfy both high strength and low yield ratio.

In general, it is well known that a yield ratio of steel is lowered by realizing a structure in which a metal structure of steel including a soft phase material such as ferrite as a major structure and a hard phase material such as bainite or martensite is appropriately distributed.

To acquire a structure in which a hard phase material is appropriately distributed in the above soft phase-based refined structure, Patent Document 1 discloses a method of lowering a yield ratio via appropriate quenching and tempering in a dual phase region of ferrite and austenite. However, the method requires an additional number of thermal treatment processes in addition to a rolling manufacturing process and, thus, there is a problem in that it is inevitable to reduce productivity and to increase manufacturing costs.

Accordingly, there has been a need to develop low-yield-ratio type, high-strength steel and a manufacturing method therefor, for ensuring super high strength and low yield ratio as well as overcoming the problem in terms of reduced productivity, increased manufacturing costs, etc.

Korean Patent Publication No.10-2015-0002958 discloses a technique for providing steel having shock resistance by ensuring the low yield ratio property by controlling the fraction so as to have a composite tissue including acicular ferrite and bainitic ferrite through controlling the alloy components and controlling the process conditions. International Publication No. WO2008/054166 discloses that a steel sheet may exhibit a strength of 930MPa or more and a toughness by adding a smaller number of alloying elements compared with the conventional technique of adding a large number of alloying elements.
Korean Patent Publication No.10-2015-0052950 discloses high-strength and low-yield ratio steel for construction having 600MPa grade tensile strength and low-yield ratio of 80% or less with low temperature toughness, and discloses that a finish cooling temperature is limited to a temperature range of 500∼600°C.

### [Cited Reference]

(Patent Document 1) Japanese Patent Laid-Open Publication No. sho 55-97425

### [Invention]

### [Technical Problem]

An aspect of the present invention is to provide low-yield-ratio type, high-strength steel and a manufacturing method therefor, and in detail, low-yield-ratio type, high-strength steel and a manufacturing method therefor, for ensuring super high strength and a low yield ratio without reduction in productivity and increase in manufacturing costs.

The objective of the present invention is not limited to the above description and the following detailed description of the present invention are exemplary and explanatory and are intended to provide further explanation of the feature as claimed by one of ordinary skill in the art without undue difficulty.

### [Technical Solution]

The present invention is described in claims 1 and 4.

The objective of the present invention is not limited to the above description and various features and advantages thereof are understood will be more clearly understood from the following detailed description.

### [Advantageous Effects]

As set forth above, according to an exemplary embodiment in the present disclosure, low-yield-ratio type, high-strength steel and a manufacturing method therefor may ensure extra high strength and a low yield ratio without reduction in productivity and increase in manufacturing costs.

### [Best Mode for Invention]

Exemplary embodiments of the present invention will now be described more fully. The exemplary embodiments of present invention may, however, be embodied in many different forms and should not be construed as being limited to the embodiments set forth herein; rather, these embodiments are provided so that this disclosure will be thorough and complete, and will fully convey the concept of the feature to those skilled in the art.

Hereinafter, low-yield-ratio type, high-strength steel according to an aspect of the present invention is described in detail.

The low-yield-ratio type, high-strength steel according to an aspect of the present invention is described in claim 1.

### Carbon (C): 0.02 to 0.11 wt%

C is an important element for forming bainite or martensite and determining a size and fraction of the formed bainite or martensite.

When a content of C is greater than 0.11 wt%, low temperature toughness may be lowered and, when a content of C is less than 0.02 wt%, formation of bainite or martensite may be obstructed to degrade strength. Accordingly, content of C is 0.02 to 0.11 wt%.

For high weldability of a plate used as a steel structure for welding, an upper limit of content of C may be 0.08 wt%.

### Silicon (Si): 0.1 to 0.5 wt%

Si is an element used as a deoxidizer for enhancing strength and toughness.

When a content of Si is greater than 0.5 wt%, low temperature toughness and weldability may be lowered and thick scale is formed on a plate surface to cause gas cuttability defects, other surface cracks, and so on. On the other hand, when a content of Si is less than 0.1 wt%, a deoxidation effect may be insufficient. Accordingly, a content of Si is 0.1 to 0.5 wt% and, more particularly, 0.15 to 0.35 wt%.

### Manganese (Mn): 1.5 to 2.5 wt%

Mn may be an element useful to enhance strength via solid-solution strengthening and, thus, it is necessary to add 1.5 wt% or more of Mn. However, when a content of Mn is greater than 2.5 wt%, toughness of a welding portion may be largely lowered due to excessive increase in hardenability. Accordingly, a content of Mn is 1.5 to 2.5 wt%.

### Aluminum (Al): 0.01 to 0.06 wt%

Al may be an element that inexpensively deoxidizes molten steel and stabilizes ferrite. When a content of Al is less than 0.01 wt%, the aforementioned effect may be insufficient. On the other hand, when a content of Al is greater than 0.06 wt%, a nozzle may clog in the case of continuous casting. Accordingly, a content of Al is 0.01 to 0.06 wt%.

### Nickel (Ni): 0.1 to 0.6 wt%

Ni may be an element that simultaneously enhances strength and toughness of a parent material. According to the present invention, to acquire the aforementioned effect, 0.1 wt% or more of Ni may be added. However, Ni is an expensive element and, thus, when Ni is added in an amount greater than 0.6 wt%, economization may be reduced and weldability may be lowered. Accordingly, content of Ni is 0.1 to 0.6 %.

### Titanium (Ti): 0.01 to 0.03 wt%

Ti prevents growth of crystal grain while being reheated to largely enhance low temperature toughness and, thus, 0.01 wt% or more of Ti may be added. However, when a content of Ti is greater than 0.03 wt%, there may be a problem in terms of a reduction in low temperature toughness due to clogging of a nozzle for continuous casting or crystallization of a central portion. Accordingly, content of Ti is 0.01 to 0.03 wt%.

### Niobium (Nb): 0.005 to 0.08 wt%

Nb may be an important element for manufacturing TMCP steel and is precipitated in the form of NbC or NbCN to enhance strength of a parent material and a welding portion. Nb that is solid-solved while being reheated at high temperature prevents re-crystallization of austenite and modification of ferrite or bainite to refine a structure. Furthermore, according to the present invention, bainite may be formed even at low cooling speed when a slab is cooled after rough rolling is performed, and stability of austenite may also be enhanced when a slab is cooled after last rolling is performed and, accordingly, generation of martensite may also be facilitated in the case of cooling at low speed.

To sufficiently acquire the aforementioned effect, content of Nb may be 0.005 wt% or more. However, when a content of Nb is greater than 0.08 wt%, brittleness crack may occur at an edge of steel. Accordingly, content of Nb is 0.005 to 0.08 wt%.

### Chromium (Cr): 0.1 to 0.5 wt%

To acquire strength, Cr may be an element added to ensure strength and may enhance quenching property. To sufficient the aforementioned effect, it may be required to add 0.1% or more of Cr. However, when a content of Cr is greater than 0.5%, rigidity of a welding portion may be excessively increased and toughness may be degraded. Accordingly, content of Cr is 0.1 to 0.5%.

### Phosphorus (P): 0.01 wt% or less

P may be an element that is advantageous for enhancing strength and anti-corrosion but largely obstructs impact toughness and, thus, content of P may be advantageously lowered and, thus, an upper content limit of P is 0.01 wt%.

### Sulfur (S): 0.01 wt% or less

S may be an element that forms MnS or the like and largely obstructs impact toughness and, thus, content of S may be advantageously lowered and an upper content limit of S is 0.01 wt%.

### Boron (B): 5 to 30 wt ppm

B may be a much inexpensive element indicating high hardenability and may be an element that is largely useful to form bainite at low speed when being cooled after rough rolling is performed.

By simply adding a small amount of B, strength may be largely enhanced and, thus, 5 wt ppm or more of B may be added. However, when a content of B is greater than 30 wt ppm, Fe₂₃(CB)₆ may be formed to rather reduce hardenability and to largely reduce low temperature toughness. Accordingly, content of B is 5 to 30 wt ppm.

### Nitrogen (N): 20 to 70 wt ppm

N enhances strength but largely reduces toughness and, thus, content of N may be controlled to be 70 wt ppm or less. However, when a content of N is controlled to be less than 20 wt ppm, steel manufacturing load is increased and, thus, a lower content limit of N is 20 wt ppm.

### Calcium (Ca): 60 wt ppm or less, but more than 0 wt ppm

Ca may be used as an element that mainly prevents non-metallic inclusion of MnS and enhances low temperature toughness. However, when an excessive amount of Ca is added, Ca reacts with oxygen included in steel to generate CaO that is non-metallic inclusion and, thus, an upper content limit of Ca is 60 wt ppm.

### Tin (Sn): 5 to 50 wt ppm

Sn may be an important element for ensuring anti-corrosion.

In terms of ensuring of anti-corrosion, 5 ppm or more of Sn may be added. However, when a content of Sn is greater than 50 ppm wt%, there may be a problem in terms of a lot of amount of detects in which a scale inflates or bursts like a blister on a steel surface rather than an effect of enhancing anti-corrosion. In addition, Sn enhances strength of steel but degrades elongation and low-temperature impact toughness and, thus, an upper content limit of Sn is 50 wt ppm.

The remaining element in the present invention is iron (Fe). However, unintended impurities from a material or a surrounding environment are inevitably introduced and, thus, the impurities are not capable of being disregarded. These impurities are known to one of ordinary skill in the art in a common manufacturing process and, thus, information on the impurities is not described throughout this specification.

Steel with the aforementioned advantageous steel composition may have a sufficient effect by simply including an alloy element with the aforementioned content range but properties such as strength and toughness of steel, and toughness and weldability of a welding heat affected zone may be further enhanced by further including one or more of 0.1 to 0.5 wt% of copper (Cu), 0.15 to 0.3 wt% of molybdenum (Mo), and 0.005 to 0.3 wt% of vanadium (V).

### Copper (Cu): 0.1 to 0.5 wt%

Cu is an element that minimizes reduction in toughness of a parent material and, simultaneously, enhances strength. To acquire the aforementioned effect, Cu of 0.1 wt% or more may be added. However, when a content of Cu is greater than 0.5 wt%, product surface properties may be largely degraded. Accordingly, content of Cu is 0.1 to 0.5 wt%.

### Molybdenum (Mo): 0.15 to 0.3 wt%

Even if a small amount of Mo is added, hardenability may be largely enhanced to enhance strength and, thus, it may be required to add 0.15 wt% or more of Mo. However, when Mo is added in an amount greater than 0.3 wt%, rigidity of a welding portion may be excessively increased and toughness may be degraded. Accordingly, a content of Mo is 0.15 to 0.3 wt% .

### Vanadium (V): 0.005 to 0.3 wt%

V is solid-solved at lower temperature than other refined alloy and is precipitated in a welding heat affected zone and prevent reduction in strength. To sufficiently acquire the aforementioned effect, 0.005 wt% or more of V may be added. However, when a content of V is greater than 0.3 wt%, toughness may be rather reduced. Accordingly, content of V is 0.005 to 0.3 wt%.

The refined structure of the steel according to the present invention includes bainitic ferrite and granular bainite in a primary phase and include M-A (martensite austenite constituent) in a secondary phase.

Bainitic ferrite includes many high tilt boundaries in a grain while maintaining an initial austenite crystal grain system and, thus, may be useful to enhance strength and impact toughness by virtue of a crystal grain refining effect.

Granular bainite maintains an initial austenite crystal grain like bainitic ferrite but a secondary phase such as M-A is present in a grain or a grain boundary. A high tilt boundary is not present in a grain boundary and, thus, it is disadvantageous for impact toughness but a large amount of low tilt boundaries are present like inter-grain electric potential and, thus, strength is slightly increased.

Bainitic ferrite and granular bainite are included in a primary phase and, thus, a low yield ratio and high strength may be ensured.

In this case, in terms of an area fraction, the bainitic ferrite is 80 to 95%, the granular bainite is 5 to 20%, and the M-A may be 3% or less.

When an area fraction of bainitic ferrite is less than 80%, it may be difficult to ensure high tensile strength and, when the area fraction is greater than 95%, there is a problem in terms of an increased yield ratio.

When an area fraction of granular bainite is less than 5%, yield strength as well as tensile strength may be increased and, thus, it is not possible to ensure a low yield ratio and, when the area fraction is greater than 20%, it may not be possible to effectively refine an initial coarsened austenite crystal grain and, thus, tensile strength may be degraded.

A secondary phase such as M-A is a refined structure useful to achieve a low yield ratio and, thus, it has an area fraction of 3% or less. When the area fraction of M-A is greater than 3%, a yield ratio may be reduced but this may function as an initiation point of cracking with respect to external stress and, thus, it may adversely affect ensuring of tensile strength.

PImax.(111)/PImax.(100) of steel according to the present invention may be 1.0 or more or 1.8 or less. The PImax. (111) may be pole intensity (PImax.) of (111) crystalline surface acquired using a method such as X-ray diffraction or electron backscatter diffraction and the PImax.(100) may be pole intensity (PImax.) of a (100) crystalline surface.

The pole intensity of the crystalline surface may be determined depending on a last refined structure of steel according to an aspect of the present invention . When bainitic ferrite and granular bainite are in a primary phase, as a fraction of bainitic ferrite is increased, a value of the PImax. (111) is increased and, as a fraction of granular bainite is increased, a value of the PImax. (100) may be increased. According to an aspect of the present disclosure, the last refined structure of the steel has bainitic ferrite with a higher area fraction than granular bainite and, when PImax. (111)/PImax. (100) is equal to or less than 1.8, it may be possible to manufacture low-yield-ratio type, high-strength steel and, when PImax.(111)/PImax.(100) is greater than 1.8, a low yield ratio may not be satisfied and, thus, an upper limit may be 1.8 or less. In detail, PImax. (111)/PImax. (100) may be 1.6 or less.

When PImax. (111) /PImax. (100) is less than 1.0, a fraction of granular bainite is increased to be greater than 20% and, thus, there is a problem in that it is difficult to ensure high strength. Accordingly, a lower limit of PImax. (111) /PImax. (100) may be equal to or greater than 1.0 and, in more detail, may be 1.2 or more.

The steel according to the present invention has a yield ratio of 0.85 or less and ensures tensile strength of 800 MPa or more and, thus, the steel may be used as steel for construction, or the like.

The steel according to the present disclosure may have a thickness of 60 mm or less.

Since the steel according to the present invention ensures high strength and a low yield ratio, the steel may have a plate thickness of 60 mm or less and, thus, it may be easy to perform machining such as cutting or perforation and a welding operation. Accordingly, the steel may have a thickness of 60 mm or less. In more detail, the thickness may be 40 mm or less and, more particularly, 30 mm or less.

A lower thickness limit of the steel may not be particularly limited but may be 15 mm or more to use the steel as steel for a construction structure.

Hereinafter, a manufacturing method of low-yield-ratio type, high-strength steel according to another aspect of the present disclosure is described in detail.

The manufacturing method of low-yield-ratio type, high-strength steel according to another aspect of the present invention may include heating a slab with the aforementioned alloy composition at 1050 to 1250°C, rough-rolling the heated slab at 950 to 1150°C to obtain a bar, hot-rolling the bar at final rolling temperature of 700 to 950 °C to acquire hot rolled steel, and cooling the hot rolled steel at cooling speed of 25 to 50°C /s up to cooling termination temperature of Bs or less.

### Heating Slab

A slab having the aforementioned alloy composition is heated to a temperature of 1050 to 1250°C.

### Rough Rolling

The heated slab is rough-rolled at 950 to 1050°C to acquire a bar.

When the rough rolling temperature is less than 950°C, as austenite is deformed in a state in which re-crystallization does not occur, there is a concern of coarsening of particles and, when the rough rolling temperature is greater than 1050°C, re-crystallization occurs and, simultaneously, particles are grown and, thus, there is also a concern of coarsening of austenite particles.

### Hot-rolling

The bar is hot-rolled at final rolling temperature of 700 to 950°C to acquire hot rolled steel.

When the final rolling temperature is less than 700°C, a temperature of a plate is low and, thus, a load is generated in a rolling mill and there is a concern in that the plate is not capable of being rolled to a final thickness and, when the final rolling temperature is greater than 950°C, there is a concern of re-crystallization during rolling.

In this case, a reduction ratio of the hot rolling is 50 to 80%.

When the final rolling reduction ratio is less than 50%, load applied to a material is increased during rolling and there is danger of facility accidents and, when the final rolling reduction ratio is greater than 80%, the number of rolling paths is increased and, thus, there is a concern of not ensuring a final thickness up to rolling termination temperature.

### Cooling

The hot rolled steel is cooled at cooling speed of 25 to 50°C/s up to cooling termination temperature of Bs or less.

When cooling of the hot rolled steel is terminated at temperature greater than Bs, a phase of bainitic ferrite and granular bainite is not sufficiently transitioned and, thus, strength is not capable of being ensured. A cooling speed has a physical limit depending on a plate thickness but, as soft ferrites are generated at a cooling speed less than 25°C/s, it may be difficult to satisfy tensile strength of 800 MPa or more. As the possibility that martensite which is low temperature transformed structure is generated at cooling speed greater than 50°C/s is high, yield strength as well as tensile strength is also increased and, thus, it may be difficult to satisfy a yield ratio of 0.85 or less.

### [Mode for Invention]

Hereinafter, the present invention will be described in detail by explaining exemplary embodiments. However, the features of the present invention will be more clearly understood and should not be limited by the exemplary embodiments of the present invention . The scope of the present invention should be determined by the appended claims and their equivalents coming within the meaning of the appended claims are intended to be embraced therein.

A slab that satisfies a component system shown in Table 1 below was heated to 1160°C , was rough-rolled at 1000°C and, then, was hot-rolled and cooled to satisfy a manufacturing condition shown in Table 2 below to acquire steel. The yield strength, tensile strength, yield ratio, and refined structure of the steel were measured and shown in Table 3 below.

In addition, pole strength of (100) and (110) crystalline surfaces of the steel was measured to obtain a value of PImax. (111)/PImax. (100) and the value was shown in Table 3 below.

The yield strength and the tensile strength were measured using a universal tensile tester.

A refined structure was obtained by mirror-like grinding the steel and, then, performing chemical corrosion and, then, was observed by an optical microscope.

Pole strength and entire structure strength were measured via an X-ray diffractometer and an electron backscatter diffractometer.

A unit of content of each element is wt% in Table 1 below.

**Table 1**

| Steel Type | C | Si | Mn | P | S | Al | Cr | Ni | Ti | Nb | B | N | Ca | Sn |
|---|---|---|---|---|---|---|---|---|---|---|---|---|---|---|
| Invention steel A | 0.045 | 0.17 | 2.12 | 0.007 | 0.002 | 0.029 | 0.32 | 0.40 | 0.018 | 0.04 | 0.0016 | 0.0037 | 0.0010 | 0.0008 |
| Invention steel B | 0.052 | 0.15 | 2.48 | 0.008 | 0.001 | 0.026 | 0.30 | 0.15 | 0.016 | 0.04 | 0.0015 | 0.0035 | 0.0007 | 0.0042 |
| Invention steel C | 0.065 | 0.16 | 1.75 | 0.011 | 0.001 | 0.030 | 0.29 | 0.29 | 0.019 | 0.04 | 0.0014 | 0.0029 | 0.0012 | 0.0021 |
| Invention steel D | 0.054 | 0.25 | 2.29 | 0.007 | 0.002 | 0.030 | 0.31 | 0.50 | 0.011 | 0.03 | 0.0013 | 0.0042 | 0.0005 | 0.0034 |
| Comparison Steel E | 0.045 | 0.11 | 1.91 | 0.005 | 0.003 | 0.006 | 0.04 | 1.52 | 0.008 | 0.01 | 0.0001 | 0.0040 | 0.0011 | 0.0004 |
| Comparison Steel F | 0.049 | 0.15 | 2.85 | 0.009 | 0.002 | 0.029 | 0.28 | 0.41 | 0.018 | 0.03 | 0.0015 | 0.0040 | 0.0014 | 0.0003 |

**Table 2**

| Steel type | Division | Hot final rolling | | Cooling | | Bs Temperature (°C) | | | | | | | | |
|---|---|---|---|---|---|---|---|---|---|---|---|---|---|---|
| | | Temperature (°C) | Reduction Ratio (%) | Cooling Speed (°C/s) | Termination Temperature (°C) | | | | | | | | | |
| Invention steel A | Invention Example 1 | 844 | 75 | 46.6 | 523 | 589 | | | | | | | | |
| | Invention Example 2 | 860 | 70 | 41.1 | 537 | | | | | | | | | |
| | Invention Example 3 | 892 | 60 | 40.6 | 492 | | | | | | | | | |
| Invention steel E | Invention Example4 | 873 | 70 | 41.2 | 536 | 565 | | | | | | | | |
| | Invention Example5 | 890 | 60 | 37.7 | 506 | | | | | | | | | |
| | Invention Example6 | 901 | 60 | 26.2 | 441 | | | | | | | | | |
| Invention steel C | Invention Example 7 | 899 | 60 | 25.8 | 451 | 623 | | | | | | | | |
| | Invention Example 8 | 890 | 60 | 26.3 | 447 | | | | | | | | | |
| | Invention Example 9 | 859 | 70 | 41.4 | 528 | | | | | | | | | |
| Invention steel D | Comparison Example 1 | 852 | 75 | 51.4 | 534 | 568 | | | | | | | | |
| | Comparison Example 2 | 863 | 75 | 57.7 | 507 | | | | | | | | | |
| | Comparison Example 3 | 904 | 45 | 6.4 | 182 | | | | | | | | | |
| Comparison Steel E | Comparison Example 4 | 870 | 72 | 34.1 | 350 | 574 | | | | | | | | |
| | Comparison Example 5 | 871 | 66 | 24.1 | 356 | | | | | | | | | |
| | Comparison Example 6 | 869 | 52 | 20.2 | 357 | | | | | | | | | |
| Comparion Steel F | Comparison Example 7 | 864 | 78 | 48.5 | 505 | 526 | | | | | | | | |
| | Comparison Example 8 | 877 | 65 | 31.4 | 502 | | | | | | | | | |
| | Comparison Example 9 | 835 | 55 | 20.4 | 496 | | | | | | | | | |

**Table 3**

| Steel Type | Division | Central portion Refined structure | | | Yield strength ( MPa) | Tensile Strength ( MPa) | Yield Ratio | PImax.(111)/ PImax.(100) |
|---|---|---|---|---|---|---|---|---|
| | | BF | GB | M.A | | | | |
| Invention Steel A | Invention Example 1 | 86 | 12 | 2 | 677 | 843 | 0.80 | 1.14 |
| | Invention Example 2 | 89 | 10 | 1 | 703 | 872 | 0.81 | 1.25 |
| | Invention Example 3 | 91 | 8 | 1 | 717 | 909 | 0.79 | 1.50 |
| Invention Steel B | Invention Example 4 | 87 | 10 | 3 | 697 | 866 | 0.80 | 1.16 |
| | Invention Example 5 | 92 | 6 | 2 | 736 | 898 | 0.82 | 1.64 |
| | Invention Example 6 | 88 | 11 | 1 | 707 | 871 | 0.81 | 1.27 |
| Invention Steel C | Invention Example 7 | 92 | 7 | 1 | 761 | 919 | 0.83 | 1.52 |
| | Invention Example 8 | 93 | 7 | 0 | 786 | 926 | 0.85 | 1.71 |
| | Invention Example 9 | 83 | 15 | 2 | 686 | 860 | 0.80 | 1.10 |
| Invention Steel D | Comparison Example 1 | 97 | 3 | 0 | 797 | 931 | 0.86 | 1.98 |
| | Comparison Example 2 | 98 | 2 | 0 | 893 | 981 | 0.91 | 1.96 |
| | Comparison Example 3 | 71 | 24 | 5 | 613 | 780 | 0.79 | 0.87 |
| Comparison Steel E | Comparison Example 4 | AF: 72, B: 28 | | | 562 | 694 | 0.81 | 1.08 |
| | Comparison Example 5 | AF: 79, B: 21 | | | 530 | 643 | 0.82 | 1.05 |
| | Comparison Example 6 | AF: 74, B: 26 | | | 504 | 612 | 0.82 | 1.07 |
| Comparison Steel F | Comparison Example 7 | BF: 97, GB: 3, MA: 0 | | | 876 | 984 | 0.89 | 1.97 |
| | Comparison Example 8 | BF: 72, GB: 24, MA: 4 | | | 725 | 841 | 0.86 | 0.85 |
| | Comparison Example 9 | BF: 66, GB: 31, MA: 3 | | | 660 | 776 | 0.85 | 0.82 |

In Table 3 above, BF is bainitic ferrite, GB is granular bainite, MA is martensite austenite constituent, AF is accicular ferrite, and B is bainite and their unit is area%.

It may be seen that Invention Examples 1 to 9 that satisfy the alloy composition and manufacturing condition according to the present invention are capable of ensuring a low yield ratio of 0.85 or less and tensile strength of 800 MPa or more.

On the other hand, Comparison Examples 1 to 3 satisfy the alloy composition according to the present invention but do not satisfy the manufacturing condition and, thus, it may be seen that a low yield ratio is not capable of being ensured or tensile strength is degraded.

Comparison Examples 4, 7, and 8 satisfy the manufacturing condition according to the present invention but do not satisfy the alloy composition and, thus, it may be seen that a low yield ratio is not capable of being ensured.

While the present invention has been described referring to the exemplary embodiments of the present invention, those skilled in the art will appreciate that many modifications and changes can be made to the present invention without departing from the essential characteristics of the present invention.

## Claims

1. Low-yield-ratio type, high-strength steel comprising:
0.02 to 0.11 wt% of carbon (C);
0.1 to 0.5 wt% of silicon (Si);
1.5 to 2.5 wt% of manganese (Mn);
0.01 to 0.06 wt% of aluminum (Al);
0.1 to 0.6 wt% of nickel (Ni);
0.01 to 0.03 wt% of titanium (Ti);
0.005 to 0.08 wt% of niobium (Nb);
0.1 to 0.5 wt% of chromium (Cr);
0.01 wt% or less of phosphorus (P);
0.01 wt% or less of sulfur (S);
5 to 30 wt ppm of boron (B);
20 to 70 wt ppm of nitrogen (N);
50 wt ppm or less, but more than 0 wt ppm, of calcium (Ca) ;
5 to 50 wt ppm or less of tin (Sn);
iron (Fe) as a remainder thereof; and
other inevitable impurities,
wherein the steel optionally further comprises one or more of 0.1 to 0.5 wt% of copper (Cu), 0.15 to 0.3 wt% of molybdenum (Mo), and 0.005 to 0.3 wt% of vanadium (V),
wherein a refined structure of the steel includes bainitic ferrite and granular bainite in a primary phase and includes M-A in a secondary phase, and
wherein the bainitic ferrite has an area fraction of 80 to 95%, the granular bainite has an area fraction of 5 to 20%, and the M-A has an area fraction of 3% or less
wherein the steel has a yield ratio of 0.85 or less and has tensile strength of 800 MPa or more.

2. The low-yield-ratio type, high-strength steel of claim 1, wherein PImax. (111) /PImax. (100) as a ratio of pole intensity (PImax.) of (100) and (111) crystalline surfaces of the steel is 1.0 or more or 1.8 or less where the PImax. (111) is pole intensity of the (111) crystalline surface and the PImax. (100) is pole intensity of the (100) crystalline surface, and is determined depending on the last refined structure of the steel.

3. The low-yield-ratio type, high-strength steel of claim 1, wherein the steel has a thickness of 60 mm or less.

4. A method of manufacturing the low-yield-ratio type, high-strength steel of claim 1, the method comprising:
heating a slab having an alloy composition as defined in claim 1 at 1050 to 1250°C ;
rough-rolling the heated slab at 950 to 1050°C to acquire a bar;
hot-rolling the bar at final rolling temperature of 700 to 950°C to acquire hot rolled steel; and
cooling the hot rolled steel at cooling speed of 25 to 50°C/s up to cooling termination temperature of Bs or less,
wherein the slab optionally further comprises one or more of 0.1 to 0.5 wt% of copper (Cu), 0.15 to 0.3 wt% of molybdenum (Mo), and 0.005 to 0.3 wt% of vanadium (V) and
wherein the hot-rolling is performed at a reduction ratio of 50 to 80%.

## Patentansprüche

1. Hochfester Stahl von der Art mit niedrigem Fließverhältnis, umfassend:
0,02 bis 0,11 Gew.-% Kohlenstoff (C);
0,1 bis 0,5 Gew.-% Silizium (Si);
1,5 bis 2,5 Gew.-% Mangan (Mn);
0,01 bis 0,06 Gew.-% Aluminium (Al);
0,1 bis 0,6 Gew.-% Nickel (Ni);
0,01 bis 0,03 Gew.-% Titan (Ti);
0,005 bis 0,08 Gew.-% Niob (Nb);
0,1 bis 0,5 Gew.-% Chrom (Cr);
höchstens 0,01 Gew.-% Phosphor (P);
höchstens 0,01 Gew.-% Schwefel (S);
5 bis 30 Gew.-ppm Bor (B);
20 bis 70 Gew.-ppm Stickstoff (N);
höchstens 50 Gew.-ppm, jedoch mehr als 0 Gew.-ppm Calcium (Ca);
höchstens 5 bis 50 Gew.-ppm Zinn (Sn);
Eisen (Fe) als ein Rest davon; und
andere unvermeidliche Verunreinigungen, wobei der Stahl optional ferner von 0,1 bis 0,5 Gew.-% Kupfer (Cu), 0,15 bis 0,3 Gew.-% Molybdän (Mo) und/oder 0,005 bis 0,3 Gew.-% Vanadium (V) umfasst, wobei die verfeinerte Struktur des Stahls bainitischen Ferrit und körnigen Bainit in einer Primärphase beinhaltet und M-A in einer Sekundärphase beinhaltet, und wobei der bainitische Ferrit einen Flächenanteil von 80 bis 95 % aufweist, der körnige Bainit einen Flächenanteil von 5 bis 20 % aufweist und der M-A einen Flächenanteil von höchstens 3 % aufweist, wobei der Stahl ein Fließverhältnis von höchstens 0,85 aufweist und eine Zugfestigkeit von wenigstens 800 MPa aufweist.

2. Hochfester Stahl von der Art mit niedrigem Fließverhältnis nach Anspruch 1, wobei PImax. (111) /PImax. (100) als Verhältnis der Polintensität (PImax.) von (100) und (111) Kristalloberflächen des Stahls wenigstens 1,0 oder höchstens 1,8 beträgt, wobei der Plmax. (111) die Polintensität der (111) Kristalloberfläche ist und der PImax. (100) die Polintensität der (100) Kristalloberfläche ist und in Abhängigkeit von der zuletzt verfeinerten Struktur des Stahls bestimmt ist.

3. Hochfester Stahl von der Art mit niedrigem Fließverhältnis nach Anspruch 1, wobei der Stahl eine Dicke von höchstens 60 mm aufweist.

4. Verfahren zum Herstellen des hochfesten Stahls von der Art mit niedrigem Fließverhältnis nach Anspruch 1, wobei das Verfahren umfasst:
Erhitzen einer Platte, die eine Legierungszusammensetzung nach Anspruch 1 bei 1050 bis 1250 °C aufweist;
Grobwalzen der erhitzten Platte bei 950 bis 1050 °C, um einen Stab zu erhalten;
Warmwalzen des Stabs bei einer Endwalztemperatur von 700 bis 950 °C, um warmgewalzten Stahl zu erhalten; und
Abkühlen des warmgewalzten Stahls mit einer Abkühlgeschwindigkeit von 25 bis 50 °C/s bis zu einer Abkühltemperatur von höchstens Bs, wobei die Platte optional ferner von 0,1 bis 0,5 Gew.-% Kupfer (Cu), 0,15 bis 0,3 Gew.-% Molybdän (Mo) und/oder 0,005 bis 0,3 Gew.-% Vanadium (V) umfasst, und wobei das Warmwalzen bei einem Reduktionsverhältnis von 50 bis 80 % durchgeführt wird.

## Revendications

1. Acier à haute résistance de type à faible rapport d'élasticité, comprenant :
0,02 à 0,11 % en poids de carbone (C) ;
0,1 à 0,5 % en poids de silicium (Si) ;
1,5 à 2,5 % en poids de manganèse (Mn) ;
0,01 à 0,06 % en poids d'aluminium (Al) ;
0,1 à 0,6 % en poids de nickel (Ni) ;
0,01 à 0,03 % en poids de titane (Ti) ;
0,005 à 0,08 % en poids de niobium (Nb) ;
0,1 à 0,5 % en poids de chrome (Cr) ;
0,01 % en poids ou moins de phosphore (P) ;
0,01 % en poids ou moins de soufre (S) ;
5 à 30 ppm en poids de bore (B) ;
20 à 70 ppm en poids d'azote (N) ;
50 ppm en poids ou moins, mais plus de 0 ppm en poids de calcium (Ca) ;
5 à 50 ppm en poids ou moins d'étain (Sn) ;
du fer (Fe) comme reste de celui-ci ; et
d'autres impuretés inévitables,
dans lequel l'acier comprend éventuellement en outre 0,1 à 0,5 % en poids de cuivre (Cu), et/ou 0,15 à 0,3 % en poids de molybdène (Mo) et/ou 0,005 à 0,3 % en poids de vanadium (V),
dans lequel une structure affinée de l'acier comporte de la ferrite bainitique et de la bainite granulaire en une phase primaire et comporte du M-A en une phase secondaire, et
dans lequel la ferrite bainitique a une fraction de surface de 80 à 95 %, la bainite granulaire a une fraction de surface de 5 à 20 %, et le M-A a une fraction de surface de 3 % ou moins,
dans lequel l'acier a un rapport d'élasticité de 0,85 ou moins et une résistance à la traction de 800 MPa ou plus.

2. Acier à haute résistance de type à faible rapport d'élasticité selon la revendication 1, dans lequel PImax. (111)/PImax. (100), comme rapport de l'intensité polaire (PImax.) de surfaces cristallines (100) et (111) de l'acier est de 1,0 ou plus, ou de 1,8 ou moins, où la PImax. (111) est l'intensité polaire de la surface cristalline (111) et la PImax. (100) est l'intensité polaire de la surface cristalline (100) et est déterminée en fonction de la dernière structure affinée de l'acier.

3. Acier à haute résistance de type à faible rapport d'élasticité selon la revendication 1, dans lequel l'acier a une épaisseur de 60 mm ou moins.

4. Procédé de fabrication de l'acier à haute résistance de type à faible rapport d'élasticité selon la revendication 1, le procédé comprenant :
le chauffage d'une brame ayant une composition d'alliage telle que définie dans la revendication 1 entre 1 050 et 1 250° C ;
le laminage grossier de la brame chauffée de 950 à 1 050° C pour obtenir un lingot ;
le laminage à chaud du lingot à une température de laminage finale de 700 à 950° C pour obtenir de l'acier laminé à chaud ; et
le refroidissement de l'acier laminé à chaud à une vitesse de refroidissement de 25 à 50° C/s jusqu'à une température de terminaison de refroidissement de Bs ou moins,
dans lequel la brame comprend éventuellement en outre 0,1 à 0,5 % en poids de cuivre (Cu), et/ou 0,15 à 0,3 en poids de molybdène (Mo) et/ou 0,005 à 0,3 % en poids de vanadium (V) et
dans lequel le laminage à chaud est effectué selon un rapport de réduction de 50 à 80 %.
